

# UNITED STATES PATENT OFFICE.

JOHN A. SCHAEFFER, OF JOPLIN, MISSOURI, ASSIGNOR TO PICHER LEAD COMPANY,  
OF JOPLIN, MISSOURI, A CORPORATION OF MISSOURI.

## ORANGE MINERAL AND METHOD OF MANUFACTURING SAME.

1,187,933.

Specification of Letters Patent. Patented June 20, 1916.

No Drawing.

Application filed September 24, 1915. Serial No. 52,465.

To all whom it may concern:

Be it known that I, JOHN A. SCHAEFFER, a citizen of the United States of America, residing in the city of Joplin, in the county 5 of Jasper, State of Missouri, have invented a certain new and useful Improvement in Orange Mineral and Method of Manufacturing Same, of which the following is a true and exact description.

10 My invention relates to the manufacture of a commercially new variety of lead tetroxid,  $Pb_3O_4$ , which by reason of its color and many of its physical characteristics, may properly be called orange mineral, but 15 which differs from the known orange mineral of commerce in that it has a much finer state of division and a considerably less weight per unit of bulk and I believe both the material and method of manufacturing

20 the same to be new with me.

Heretofore orange mineral which, although chemically the same, is distinguished from red lead by its color and texture, has been made by the decomposition of corroded 25 white lead, and the subsequent re-oxidation of this product, and my invention is based on my discovery that a product having the color peculiarities of and an even finer amorphous texture than the orange mineral 30 heretofore known, can be manufactured by subjecting volatilized or fumed litharge to an oxidizing calcination which will convert the monoxid into tetroxid and my invention accordingly consists, in the first place, in 35 the method of manufacturing my new orange mineral which consists in subjecting volatilized or fumed litharge to an oxidizing calcination at a proper temperature, which I have ascertained to be approxi- 40 mately 850° F. and, in the second place, my invention consists in the new orange mineral manufactured from the volatilized litharge and characterized by a finer state of subdivision and a less weight in unit of bulk 45 than previously known varieties of orange mineral.

The substance I have referred to as volatilized litharge is the product of the volatilization of melted litharge, monoxid of 50 lead, condensed and collected, preferably by passing the volatilized oxid through a cooling system and finally into a bag room where the condensed oxid fume is separated from the furnace gases. For this purpose

apparatus similar to that employed in the 55 manufacture of "sublimed white lead" is conveniently employed.

The oxidation of the volatilized or fumed litharge is conveniently carried on in ordinary types of reverberatory furnaces such 60 as are used in the manufacture of red lead and orange mineral from massicot and the product of decomposed white lead or lead carbonate. I have found in practice that a temperature of approximately 850° F. 65 gives the best result. The oxidation will of course take place at lower temperatures with less speed and it is necessary to avoid a temperature so high as to tend to reconvert the tetroxid into litharge. It will be understood that the mass should be stirred by any 70 convenient means to promote the rapidity of the oxidation.

The color of the product obtained from the volatilized litharge in the manner described will depend on the percentage of  $Pb_3O_4$  in the finished product which may be varied, as in previously known methods of manufacturing orange mineral, by varying the period to which the material is subjected to the oxidizing calcination, but in all cases the texture of the new orange mineral will be found to be finer than that of the orange mineral manufactured before the herein described orange mineral was discovered, and its weight per cubic inch materially less.

I have found that a cubic inch of my new orange mineral will weigh from 9 to 11 grams while orange mineral as heretofore 90 made by old methods will weigh from 20 to 25 grams per cubic inch. The fineness of division of my new orange mineral in comparison with the older products of orange mineral bears about the same ratio which 95 all pigments formed by a fumed process bears to pigments which are mechanically ground, it is not possible to get even an approximate state of sub-division by mechanical grinding as compared with the subdivision secured by a fume process. The great difference in fineness results in the important practical advantage that with my new orange mineral 12 to 14 pounds ground in oil will give a paint of proper painting 100 consistency while the older orange minerals of coarser consistency must be used in the proportion of 20 to 24 pounds to a gallon 105

of oil to produce a paint of the same painting consistency.

The gram weights per cubic inch referred to above are those obtained by the use of the Scott volumeter with the Schaeffer-White modification in the regularly prescribed operation of this volumeter. While the orange mineral prepared by this process shows a gram weight and fineness as above stated, it would be possible to vary the fineness to a certain extent by changing the settling system so as to obtain either a finer or a coarser fumed litharge which would of course result in a finer or coarser orange mineral with greater or less weight per cubic weight and a corresponding change in the weight required to give a paint of the proper painting consistency.

Having now described my invention, what

I claim as new and desire to secure by Letters Patent, is:—

1. The method of manufacturing orange mineral which consists in subjecting finely divided litharge, obtained by volatilizing litharge and collecting the condensed fume, to calcination in an oxidizing atmosphere at a temperature of approximately 850° Fahrenheit.

2. As a new article of manufacture orange mineral formed by calcination of litharge finely divided by volatilization, said orange mineral being characterized by a finer division and less weight per unit of bulk than known varieties of orange mineral made by the decomposition of corroded white lead and its subsequent reoxidation.

JOHN A. SCHAEFFER.